

2,782,117

## METHOD OF RECLAIMING URANIUM

Harley A. Wilhelm, Ames, Iowa, and C. F. Gray, Baton Rouge, La., assignors to the United States of America as represented by the United States Atomic Energy Commission

No Drawing. Application June 5, 1946,  
Serial No. 674,648.

4 Claims. (Cl. 75—84.1)

This invention relates to the reclamation of uranium filings and turnings from the waste of metallurgical operations with uranium and recasting the reclaimed uranium. The reclamation of uranium from waste turnings and filings is complicated by the necessity of achieving a product of a high degree of purity and also complicated by the high affinity of this metal for oxygen.

An object of this invention is the recasting of uranium from reclaimed uranium waste.

Another object of this invention is the provision of a process for reclaiming uranium from uranium waste and casting the reclaimed uranium with a suitable reducing metal, such as for example, an alkali or alkaline earth metal, to form a uranium casting with the minimum of oxidation and a high degree of purity.

The above and other objects and features of this invention will be apparent from the following detailed description of a preferred embodiment.

In casting reclaimed uranium, it has been discovered that highly satisfactory results are obtained by the inclusion of an alkali or an alkaline earth metal in the melt. According to this method the uranium may be processed from any condition in uranium waste to pure uranium billets with a high percentage recovery of uranium and a minimum of oxidation.

In preparing the waste uranium for reclamation, the scrap metal is sorted and searched for relatively large pieces of foreign material which are removed by hand. The sorted uranium waste is then cut or shredded by known methods, cleaned and then re-examined for foreign material. The uranium thus processed, is then mixed with a suitable alkali or alkaline earth metal and pressed into billets for casting into biscuits or ingots.

The process generally involves the steps of sorting the uranium waste and separating out foreign matter by inspection and magnetic attraction, followed by passing the metal through a cutter in which a cleaning solution acts as a coolant and also serves to partially degrease and clean the uranium pieces. The steps after cutting involve the further cleaning and degreasing of the cut uranium in a cleaning machine followed by centrifugal drying in a stream of warm air, after which the cleaned uranium cuttings are subjected to re-examination for foreign matter. The final step in the preparation for casting entails pressing the reclaimed uranium with the desired reducing metal.

As examples of suitable reducing metals there may be mentioned sodium, barium, potassium, magnesium, calcium, and the like.

According to a preferred mode of operation of this invention uranium turnings, borings, chips, or other uranium wastes are sorted and separated for examination and removal of foreign matter and then the uranium bodies are subjected to the action of a magnetic separator to remove iron or steel therefrom. A magnetic separation is important to protect the cutter in the next stage of operation from large pieces of iron and steel.

The uranium particles are next cut and in this stage the inspected uranium is placed in a spray containing a wetting agent and a suitable detergent, such as a 3% solution of sodium silicate. Such a spray is directed so as to follow the uranium particles into the cutter. The cutting is preferably done by a hammer-type mill to give an optimum amount of abrasive and bending action to the particles and thereby remove the oxide scale. The uranium turnings should be cut only fine enough that the particles will flow from one container to another without hanging together objectionably.

The 3% silicate solution mentioned above is highly satisfactory in that it serves both as a coolant and as a degreasing agent. However, any suitable detergent solution or high flash-point, non-reactive liquid or solution may be used as a coolant in the cutting operation. In any event cutting the uranium should be conducted while the uranium is wetted and cooled with a liquid coolant in order to prevent fire.

The next step in the process is that of washing the uranium particles as they are delivered from the cutter. The cleaning operation involves washing the uranium particles with a suitable detergent solution followed by rinsing twice in cold water. An additional step which aids in the removal of the oxide film may be employed by dipping or otherwise allowing the uranium particles to be treated with a hydrogen peroxide-sulfuric acid bath for several minutes. Such a solution attacks the oxide layer much more rapidly than it attacks the uranium metal. After the metal has been rinsed it is placed in a centrifuge equipped with a blower which forces heated (50° C.) air through the mass as it is being whirled.

An additional oxide removal step is optional. This removal may be effected by nitric acid, hydrogen peroxide in sodium carbonate, or hydrogen peroxide in sulfuric acid.

After removal of the cleaned particles from the final rinse the wet particles are placed in a centrifuge drier and centrifuged to remove the moisture. After draining, the particles are then separated in oven trays in layers not over  $\frac{3}{4}$  of an inch in depth and dried for 15 minutes at 60° C. in a vacuum of 20" in mercury or less.

The dried material from the vacuum drying oven is deposited on a sorting belt and slowly passed along by the sorting belt in a thin layer so that the sorting operator may remove small pieces of non-magnetic material. The uranium particles are then passed over a spout-type magnetic separator for final separation after which the uranium is ready to be pressed.

Applicants have found that the yield of uranium may be substantially improved by melting the cleaned uranium with a small amount of alkali metal or alkaline earth metal. Use of as little as 0.05 to 0.1 percent by weight of such a metal based upon the weight of uranium improves the yield of uranium by several percent. Higher amounts of the alkali or alkaline earth metal may be used although such excesses are unnecessary. The amount of such metal used is almost never as much as 5 percent of the weight of the uranium and in general is below one percent.

In the case of magnesium, for example, the dried uranium particles are mixed with the magnesium in proportions of about 1 part by weight of magnesium to 1000 parts by weight of uranium and are pressed into briquettes which can be handled easily. The pressed briquettes are then melted and cast in standard casting equipment for the regular casting of crude metal biscuits. The maximum casting temperature should be about 1350° to 1375° C. and the molten metal should be poured at from about 1280° to 1300° C.

From the foregoing it will be seen that an improved

method of reclaiming uranium from waste material has been discovered, comprising cleaning and degreasing the uranium and casting the cleaned uranium with magnesium or other suitable alkali or alkaline earth metals.

What is claimed is:

1. In a process for the reclamation of uranium metal from compositions comprising uranium metal particles partially coated with an oxide scale surface, the steps which comprise contacting the uranium particles with an oxide scale-removing solution, removing said solution therefrom, intimately admixing magnesium metal with the uranium particles to form a mixture thereof, compressing said mixture into briquettes, smelting said compositions and the magnesium metal within a temperature from about 1250° C. to about 1400° C., and then casting the uranium metal within a temperature range from about 1280° C. to about 1300° C.

2. The process of claim 1 wherein the oxide scale-removing solution contains a solution of hydrogen peroxide and sulfuric acid.

3. A process for reclaiming uranium from waste metal particles comprising washing the particles with a detergent, rinsing said particles with water to remove adhering detergent, immersing the particles into an oxide-removing solution, drying the particles, mixing said particles with from 0.05 to 1% of a metal selected from the group consisting of alkali metals and alkaline earth metals, melting and heating the mixture to from 1350° to 1375° C., and pouring the metal into a mold at a temperature between 1280° and 1300° C.

4. A process for reclaiming uranium from waste metal particles comprising washing the particles with a detergent, rinsing said particles with water to remove adhering detergent, immersing the particles into a mixture of hydrogen peroxide and sulfuric acid to remove any oxide, rinsing with water, drying the particles, mixing said particles with from 0.05 to 0.1% of a metal selected from the group consisting of alkali metals and alkaline earth metals, melting and heating the mixture to from 1350° to 1375° C., and pouring the metal into a mold at a temperature between 1280° and 1300° C.

#### References Cited in the file of this patent

#### UNITED STATES PATENTS

|    |           |          |               |
|----|-----------|----------|---------------|
| 15 | 1,568,685 | Moore    | Jan. 5, 1926  |
|    | 1,646,734 | Marden   | Oct. 25, 1927 |
|    | 1,659,209 | Marden   | Feb. 14, 1928 |
|    | 1,685,915 | Gero     | Oct. 2, 1928  |
| 20 | 2,251,088 | Zeppelin | July 29, 1941 |
|    | 2,356,329 | Lundbye  | Aug. 22, 1944 |

#### OTHER REFERENCES

Thews: Metallurgy of White Metal Scrap and Residue, published by D. Van Nostrand Co., Inc., 250 Fourth Avenue, N. Y., 1930, page 4.

Smyth, "A General Account of the Development of Methods of Using Atomic Energy for Military Purposes Under the Auspices of the U. S. Government. 1940-45. August 1945, page 27. For sale by the Superintendent of Documents, Washington, D. C.